

May 4, 1971

J. F. BLUM

3,577,355

RESISTOR COMPOSITION

Filed Dec. 21, 1967



INVENTOR.  
Jack F. Blum  
BY  
Joseph E. Kieninger  
ATTORNEY

3,577,355

**RESISTOR COMPOSITION**

Jack F. Blum, Flint, Mich., assignor to General Motors Corporation, Detroit, Mich.

Filed Dec. 21, 1967, Ser. No. 692,485

Int. Cl. H01t 13/36; H01b 1/02

U.S. Cl. 252—512

6 Claims

**ABSTRACT OF THE DISCLOSURE**

An improved resistor composition for use in resistor spark plugs and other electrical devices is disclosed. The resistor composition contains a metal powder taken from the group consisting of zinc, antimony and tellurium in addition to the conventional resistor composition ingredients. The metal, for example, zinc, causes the resistor mass to bond tightly to the center electrode head in the spark plug insulator centerbore.

This invention relates to resistors, and more particularly to glass phase semiconductor resistor compositions suitable for use in resistors and resistor spark plugs of the automotive aviation type.

Resistors are commonly used to suppress the high frequency oscillations present with spark discharge in an ignition system, the oscillations resulting in rapid erosion of the spark plug electrodes and in interference with electronic equipment. Resistor spark plugs are effective in reducing automobile radio frequency interference and are particularly useful for FM broadcast and shortwave broadcast automobile receivers.

There are two basic types of resistor compositions. One type of monolithic resistor spark plug described in the McDougal et al. Pat. No. 2,459,282 granted Jan. 18, 1949, comprises a heterogeneous mixture of conductor material, that is, carbon either alone or in combination with various conducting metals, metal oxides and metal carbides with glass. In this type of resistor the conducting material, such as carbon, exists as a continuous phase and the resistance of the resistor is dependent solely upon the amount of conductor material that is present. The glass serves only to suspend the conductor material in a rigid structure. An example of this type resistor composition consists essentially of 64 weight percent borosilicate glass, 9 weight percent magnesium borate glass, 11 weight percent fluorospar, 15% beryll and 1% thermax carbon.

The second basic type of monolithic resistor spark plug is described in the patent to Counts et al., No. 2,864,884 granted Dec. 16, 1958, and No. 3,235,655 granted Feb. 15, 1966. This type of resistor consists of a semiconductor material with glass and a small amount of reducing agent such as powdered aluminum or carbon. In this type of resistor, the semiconductor material exists as a continuous phase and the resistance of the resistor is dependent mainly upon the resistance characteristics of the semiconductor material that is present. In this type of resistor, the amount of reducing agent, that is carbon or powdered aluminum and the like, are added to obtain precision-like control of the resistance of the final product, but the amount of reducing agent added should be small so that it is present in the product in a discontinuous phase and, as a result, does not function as a conductor material but solely as a reducing agent. An example of this type of resistor composition consists essentially of 25 parts barium borate glass, 30 parts filler (mullite), 0.8 part aluminum, 0.8 part thermax carbon black, 3 parts bentonite and 45 parts of a semiconductor composition containing 60 parts  $TiO_2$ , 20 parts  $SnO_2$ , 10 parts  $Ta_2O_5$ , 4 parts  $MoO_3$  and 40 parts  $Al_2O_3$ .

These two basic types of spark plug resistors described

above have been improved by the addition of a water soluble, charable carbon containing material so that they are substantially resistant to change when subjected to electrical aging or field use. This is described fully in the copending patent application Ser. No. 670,178, assigned to the assignee of the present patent application.

All of the resistor compositions referred to above are positioned in the spark plug centerbore of a resistor spark plug between two electrical conductive glass seals.

- 5 10 One conductive glass seal bonds tightly to the center electrode head and the other conductive glass seal bonds tightly to the lower end of the terminal screw. It is necessary to use the conductive glass seals on either side of the resistor seal because the resistor seals of the type described above do not bond tightly to and maintain good contact with the center electrode head and/or the terminal wire. Resistor spark plugs employing a resistor seal position between the two electrical conductive glass seals are typically referred to as three-load resistor plugs.
- 15 20 It is the primary object of this invention to provide an improved resistor composition. It is another object of this invention to provide a resistor composition which will bond tightly to the center electrode head and maintain good contact therewith to provide a stable spark plug resistance over a long period of time. It is another object of this invention to provide a two load resistor spark plug.

25 30 These and other objects are accomplished by a resistor composition containing a metal taken from the group consisting of zinc, antimony and tellurium in addition to the conventional resistor composition ingredients. The resistor composition in accordance with this invention consists essentially of 20 to 75 weight percent glass, 15 to 80 weight percent inert filler, 0 to 60 weight percent semiconductor, 0 to 3.0 weight percent inorganic binder, 0.1 to 4.0 weight percent carbon black, 0.1 to 4.0 weight soluble, charable carbon containing material and either 2 to 15 weight percent of a metal taken from the group consisting of zinc and antimony or 0.5 to 5.0 weight percent tellurium. When a spark plug having a resistor 35 40 composition of this type positioned above and around the nickel center electrode head is heated and pressed with a terminal screw, as is the practice in the art, the resulting fused mass forms a resistor seal which bonds tightly to the center electrode head and which has a stabilized resistance for an extended period of time. The metal taken from the group consisting of zinc, antimony and tellurium alloys with the nickel center electrode head to form a metal-nickel alloy coating thereon which enable the resistor composition to bond tightly to the center electrode head thereby eliminating the need for the lower conductive glass seal normally found in the prior art three-load resistor 45 50 spark plugs.

55 Other objects and advantages of this invention will be apparent from the following detailed description, reference being made to the accompanying drawing wherein a preferred embodiment of this invention is shown.

Referring now to the drawings, the spark plug 10 comprises a conventional outer metal shell 12 having a ground electrode 14 welded to the lower end thereof. Positioned 60 within the metal shell 12 and secured in the conventional manner is the insulator 16. The ceramic insulator 16 should preferably be of a high aluminum base material containing upwards of 85% aluminum oxide such, for example, as covered by U.S. Pat. No. 2,760,875, issued to 65 Karl Schwartzwalder and Helen Blair Barlett. The insulator 16 is formed with a centerbore having a lower portion 18 of relatively small diameter and an upper portion 20 of larger diameter which are connected by the insulator centerbore ledge 22. Positioned in the lower portion 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195

coated with zinc, antimony or tellurium may be used. The center electrode 24 has an enlarged head 26 at the upper end thereof which rests on the inner insulator centerbore ledge 22 and a serrated lower end 28 thereof projecting beyond the lower tip of the insulator 16. Positioned in the upper portion 20 of the insulator centerbore is a terminal screw 30. The monolithic resistor element or seal 32 of this invention which will be hereinafter fully described is positioned in the insulator centerbore 20 and is bonded to the center electrode head 26 and to the inner walls of the ceramic insulator. The center electrode 26 has a metal coating 34 thereon which will be hereinafter also fully described. Positioned on top of the resistor seal 32 in the insulator centerbore 20 is a conductive metal-glass seal 36. The conductive metal-glass seal 36 is bonded to the terminal screw 30 and the inner walls of the ceramic insulator.

The conducting metal-glass seal 36 may be made of any suitable material capable of being bonded to the insulator and to the resistance element and possessing good electrical conductivity. We prefer to use a mixture of glass and conducting materials as described and claimed in the Schwartzwalder et al. Pats. No. 2,106,578 granted Jan. 15, 1938 and No. 2,248,415 granted July 8, 1941, in the Blum et al. Pat No. 3,349,275 granted Oct. 24, 1967 and in the copending patent application Ser. No. 563,775 assigned to the assignees of this invention. An example of a conducting metal-glass seal is a composition containing 50 parts copper powder, 14 parts zinc powder, 1 part of an organic binder such as hydrogenated cottonseed oil and 35 parts of a borosilicate glass containing 65 weight percent  $\text{SiO}_2$ , 23 weight percent  $\text{B}_2\text{O}_3$ , 5 weight percent  $\text{Al}_2\text{O}_3$ , and 7 weight percent  $\text{Na}_2\text{O}$ . The conductive glass seal 36 together with the resistor seal 32 provides an electrical conductive path from the terminal screw 30 to the center electrode 24.

In accordance with the present invention, the spark plug resistor seal 32 is a dense, fused mass containing glass, insert filler material, carbon, inorganic binder, a water soluble charable carbonaceous material and a metal taken from the group consisting of zinc, antimony and tellurium. The composition of the resistor seal 32 of our invention may be formed of the following constituents in the percent by weight noted.

|                                                                                                                               | Wt. percent          |
|-------------------------------------------------------------------------------------------------------------------------------|----------------------|
| Glass                                                                                                                         | 20 to 75             |
| Inert filler—kyanite, borolon, zirconia, mullite, chromium oxide, and the like                                                | 15 to 80             |
| Semiconductor material                                                                                                        | 0 to 60              |
| Carbon black                                                                                                                  | 0.1 to 4.0           |
| Inorganic binder—Bentonite (clay)                                                                                             | 0 to 3               |
| Water soluble charable carbon containing material—dextrin, sucrose, methyl cellulose, corn flour, polyvinyl alcohol, glycerin | 0.1 to 4.0           |
| Zinc, antimony (tellurium)                                                                                                    | 2 to 15 (0.5 to 5.0) |

The glass used in the spark plug resistor seal 34 may be any conventional glass commonly used in spark plug seals. Barium borate glasses are preferred although this invention is not limited thereto. An example of a suitable barium borate glass is a composition containing 75 weight percent  $\text{B}_2\text{O}_3$  and 25%  $\text{BaO}$ . Another barium borate glass is a composition containing 60 weight percent  $\text{B}_2\text{O}_3$ , 32 weight percent  $\text{BaO}$ , 6 weight percent  $\text{Na}_2\text{O}$  and 2 weight percent  $\text{CaO}$ . Another example is a composition containing 60 weight percent  $\text{B}_2\text{O}_3$ , 38 weight percent  $\text{BaO}$  and 2 weight percent  $\text{Na}_2\text{O}$ . It has been found that the amount of the particulate glass used has no appreciable effect on the resistance of the composition within the limits of 20 to 75 weight percent.

The fluidity of the final resistor composition, as exhibited during the hot pressing operation, is controlled by the presence of a filler which does not react chemically with the other constituents of the resistor composition. These fillers may be selected from the broad group of filler materials commonly used in resistor glass seals. Ex-

amples of suitable fillers are kyanite, alumina, zirconia, mullite, borolon and the like. A preferred filler is a mixture of 25 parts by weight kyanite and 35 parts by weight zirconia. The concentration of the filler is from about 25 to 80 weight percent.

5 Since the resistor composition is best handled in a granular form, a binder such as bentonite, a very plastic aluminum silicate, is added to bond the particles together during processing. Inorganic binders such as bentonite, as well as other clays, may be used. Organic binders are not recommended for the practice of this invention since it is well known in the art that this type of material causes the resistance of the resistor to be unstable. The concentration of the binder is from 0.0 to 3.0 weight percent.

10 The concentration of the carbon black in the resistor composition is from about 0.1 to 4.0 weight percent. The carbon black may function as the sole conductor material for resistors of the type described in the McDougal et al. Pat. No. 2,459,282 previously referred to, or solely as a reducing agent as in the resistors of the type described in the Counts et al. Pat. No. 2,864,884.

15 A water soluble, charable carbonaceous material such as dextrin, sucrose, methocel, corn flour, polyvinyl alcohol and glycerine is incorporated into the resistor mass in a concentration so that this material combines with the carbon black and/or semiconductor material to provide a resistor mass which is resistant to electrical aging. The use of water soluble, charable carbonaceous material in resistors is described in the copending patent application 20 SN 670,178 assigned to the assignees of the present invention and is incorporated herewith by reference. The concentration of the water soluble, charable carbonaceous material in the resistor composition is from about 0.1 to 4.0 weight percent.

25 It has been found that a metal powder taken from the group consisting of zinc, antimony and tellurium in a resistor composition enables the resistor mass to bond tightly to the nickel center electrode head. These metals, zinc, antimony and tellurium, have relatively low melting points which are 788° F., 1258° F. and 846° F., respectively. The melting points of these materials are lower than the temperature encountered during the assembly of the spark plug, thereby indicating that these metals are most likely in a liquid state during the pressing of the 30 terminal screw step in the assembly of the resistor plug. It is believed, although this invention is not limited to this theory, that the metal powder melts and while it is in a liquid state, it either forms a metal coating for example, zinc, or a metal alloy coating, for example, zinc-nickel on the center electrode head. A substantial portion, for example 70 to 80 percent, of the metal in the resistor composition migrates to the two ends of the composition, thereby making a portion of the metal readily available for coating the center electrode head. This coating lessens 35 oxidation of the center electrode and is wetted by the fluid glass seal more effectively during the pressing operation. As a result, a weak-to-strong bond between the resistor glass seal phase and the center electrode is formed. Resistor compositions which are substantially identical except 40 that they do not contain the metal powders referred to above do not adhere to the center electrode whereas when one of these metal powders is present, the resistor composition does adhere to the electrode. One advantage of 45 such a system is that one of the conductive glass seals can be eliminated thereby reducing the manufacturing costs. The particle size of the metal powder is not critical in the practice of this invention as long as a uniform resistor composition can be made. The concentration of the zinc or 50 antimony is 2 to 15 weight percent with the preferred concentration being about 3 to 7 weight percent. The concentration of the tellurium is 0.5 to 10.0 weight percent with the preferred concentration being 4 to 5 weight percent.

55 The resistor compositions of this invention may be prepared in granular form by first dry mixing the materials

and then adding water to make a plastic mass. The plastic mass is then forced through a 20 mesh screen and the resulting granules dried. The dried material is then regranulated through a 28 mesh screen and the material retained between 28 and 100 mesh is used. This sizing procedure has been found to produce granules which are most suitable for uniform volumetric feed in the mass production of resistor spark plugs. Alternatively, the materials may be dry mixed and formed into a free-flowing slip by the addition of water. The slip is then passed into a spray drying tower where the desired agglomerates are formed.

In assembling the spark plug 10, the center electrode 24 is positioned within the centerbore 18 of the insulator 16. The desired amount of the granulated resistor composition 32 is then placed in the centerbore on top of the center electrode head 26 and rammed, followed by a measured amount of the powdered copper-glass seal material 36 which is likewise rammed to form the upper seal 36. A terminal screw 30 is then positioned within the bore and the whole assembly is then heated to a temperature which softens the glass and chars the charable, carbonaceous material, a temperature of 1550 to 1750° being generally satisfactory. A temperature of 1675° with an 18 minutes heating cycle and a 6 to 8 minute hold at the aforementioned temperature is preferred with the barium borate glass used in the preferred embodiment. Other temperatures may be employed for glasses which soften at a lower temperature. When the glass is sufficiently softened, pressure is applied to the terminal screw 30 to force it down into the centerbore, thereby depressing the softened materials and causing the upper seal portion 36 to surround and grip the lower end of the terminal screw. By hot pressing in this manner, which is the customary manner in the art, a continuous electrical path is formed from the terminal screw 30 to the center electrode head 28 through the resistance element and the conductive seal, the portions intermediate the top of the electrode and the bottom of the screw being sealed in glass-tight relationship with the walls of the insulator of the metal parts. The thus formed insulator assembly is then assembled in the shell 12 to form plug 10.

#### EXAMPLE NO. 1

A resistor plug having a resistor seal composition containing 10.0 weight percent zinc, 26.7 weight percent glass, 43.6 weight percent zirconia, 16.7 weight percent Indian kyanite, 1.6 weight percent Thermax (carbon black), 0.4 weight percent dextrin and 1.0 weight percent borax was made by positioning the resistor composition about the center electrode head in the spark plug centerbore, placing a conventional conductive glass seal on top of the resistor composition and by pressing the terminal screw in to the resistor composition at a temperature in the range of 1500 to 1600° F. The resultant resistor spark plug was cut in half to observe the adherence of the resistor seal to the center electrode. The resistor composition adhered tightly to a zinc or a zinc-nickel coating which covered the nickel center electrode head. The good adherence was attributed to the formation of the metal coating on the center electrode head.

#### EXAMPLE NO. 2

A resistor spark plug having a resistor seal composition containing 10.0 weight percent antimony, 26.7 weight percent glass, 43.6 weight percent zirconia, 16.7 weight percent Indian kyanite, 1.6 weight percent Thermax (carbon black), 0.4 weight percent dextrin and 1.0 weight percent borax was made as described in Example No. 1. The resultant spark plug was cut in half to observe the adherence of the resistor seal to the center electrode. The resistor composition adhered tightly to an antimony or antimony-nickel coating which covered the nickel center electrode head. The good adherence was attributed to the formation of the metal coating on the center electrode head.

#### 6 EXAMPLE NO. 3

A resistor spark plug having a resistor composition containing 7.0 weight percent tellurium, 26.7 weight percent glass, 43.6 weight percent zirconia, 16.7 weight percent Indian kyanite, 1.6 weight percent Thermax (carbon black), 0.4 weight percent dextrin and 1.0 weight percent borax was made as described in Example No. 1. The resultant resistor spark plug was cut in half and it was observed that the resistor composition adhered tightly to a tellurium or a tellurium-nickel coating which covered the nickel center electrode head.

The semiconductor materials that may be used in this spark plug resistor seal are of the type described in the patent to Counts et al., No. 3,235,655 granted Feb. 15, 1966, which describes a semiconductor material formed from the binary metal oxide systems consisting of  $TiO_2$ - $ZrO_2$ ,  $Ta_2O_5$ - $ThO_2$ ,  $Ta_2O_5$ - $CeO_2$  and  $Ta_2O_5$ - $Di_2O_4$  as well as the semiconductors described in the patent to Counts et al., No. 2,864,884 granted Dec. 16, 1958, where the semiconductor material comprises titanium oxide, tin oxide, tantalum oxide, vanadium oxide, molybdenum oxide, and tungsten oxide. The concentration of the semiconductor material is from 0 to 80 weight percent. An example showing the good adherence between this type of resistor composition when it contains zinc is given below.

#### EXAMPLE NO. 4

A resistor composition containing 5 parts by weight zinc, 33 parts barium borate glass, 23 parts kyanite, 2.4 parts thermax (carbon), 2.4 parts aluminum powder, 2.8 parts bentonite and 37 parts of a stannous titanate semiconductor consisting of 44.4 weight percent titanium dioxide, 29.6 weight percent alumina, 14.8 weight percent tin oxide, 7.4 weight percent tantalum oxide and 3.7 weight percent molybdic acid was prepared and placed in the spark plug insulator centerbore around the nickel center electrode head. After the resistor spark plug was completely assembled by the same steps as previously described, the resistor spark plug was cut in half to observe the adherence of the resistor to the center electrode. This resistor spark plug had a zinc-nickel alloy coating on the center electrode head and there was good adherence between the resistor composition and the center electrode head.

These examples indicate that the metals in the group consisting of zinc, antimony and tellurium promote the formation of a metal coating on the center electrode head which results in good adherence between the resistor composition and the center electrode head.

The resistor compositions of this invention contain a metal taken from the group consisting of zinc, antimony and tellurium which enable a good bond to be formed between the resistor seal and the center electrode thereby reducing the need of a conductor glass phase about the center electrode head. The resistor spark plug of this invention has a high degree of stability when subjected to field use since good contact between the center electrode head and the resistor seal is maintained for substantially the life of the resistor spark plug.

While the invention has been described in terms of specific examples, it is to be understood that the scope of the invention is not limited thereto except as defined by the following claims.

What is claimed is:

1. A gas sealing resistance composition for use in a resistor spark plug consisting essentially of glass having a softening temperature of from 1500-1750° F., an inert filler material in the amount of at least 15% by weight and a single metal powder taken from the group of relatively low melting point metals consisting of zinc, antimony and tellurium.

2. A resistance composition as described in claim 1 wherein the concentration of said metal powder taken from the group consisting of zinc and antimony is about 2 to 15 weight percent.

3. A resistance composition as described in claim 1 wherein the concentration of said tellurium powder is about 0.5 to 10.0 weight percent.

4. A gas sealing resistance element having a tight bond with the center electrode head in a spark plug insulator centerbore, said head having a coating of relatively low melting point metal deposited thereon from the gas sealing resistance composition, formed from a composition consisting essentially of 20 to 75 weight percent glass having a softening temperature of from 1500-1750° F., 15 to 80 weight percent inert filler, 0 to 60 weight percent semiconductor material, 0.1 to 4.0 weight percent carbon black, 0 to 3 weight percent inorganic binder, 0.1 to 4.0 weight percent water soluble charable carbonaceous material and 2 to 15 weight percent of a metal powder taken from the group of relatively low melting point metals consisting of zinc and antimony, said composition having been heated in said insulator centerbore to a temperature of from 1500-1750° F. at which said metal melts a portion of said metal forming a coating on said center electrode head.

5. A resistor spark plug comprising a ceramic insulator having a centerbore therethrough, a center electrode having its head in said centerbore and a fused gas sealing resistor mass bonded to said center electrode head, said head having a coating of relatively low melting point metal deposited thereon from the gas sealing resistor composition, said resistor mass consisting essentially of glass having a softening temperature of from 1500-1750° F., an inert filler material in the amount of at least 15% by weight and a metal taken from the group of relatively

low melting point metals consisting of zinc, antimony and tellurium, a portion of said metal forming a coating on the end of said electrode bonded to said resistor mass.

6. A gas sealing resistance element having a tight bond with the center electrode head in a spark plug insulator centerbore, said head having a coating of relatively low melting point metal deposited thereon from the gas sealing resistance composition, formed from the composition consisting essentially of 20 to 40 weight percent glass having a softening temperature of from 1500-1750° F., 50 to 70 weight percent inert filler, 1 to 3 weight percent carbon black, 1 to 3 weight percent inorganic binder, 0.2 to 3 weight percent water soluble charable carbonaceous material and 5 to 10 weight percent zinc powder having a relatively low melting point, said composition having been heated in said insulator centerbore to a temperature of from 1500-1750° F. at which said zinc powder melts, a portion of said zinc forming a coating on said center electrode head.

#### References Cited

#### UNITED STATES PATENTS

|           |         |             |       |         |
|-----------|---------|-------------|-------|---------|
| 3,349,275 | 10/1967 | Blum et al. | ----- | 313-136 |
| 2,695,240 | 11/1954 | Oshry       | ----- | 106-46  |
| 3,076,908 | 2/1963  | Pfaender    | ----- | 252-512 |
| 3,226,342 | 12/1965 | Kesten      | ----- | 252-512 |

DOUGLAS J. DRUMMOND, Primary Examiner

U.S. CL. X.R.

30 106-47; 313-145